# EUROPEAN PATENT SPECIFICATION

(11) **EP 0 086 837 B1**
(45) Date of publication and mention of the grant of the patent: **27.12.1985**
(21) Application number: 81902444.9
(22) Date of filing: 27.08.1981
(51) Int. Cl.: H04R 7/02

(54) **VIBRATING PLATE FOR SPEAKER**
VIBRIERENDE PLATTE FÜR LAUTSPRECHER
MEMBRANE VIBRANTE POUR HAUT-PARLEUR

(43) Date of publication of application: 31.08.1983
(73) Proprietor: TORAY INDUSTRIES, INC., Tokyo 103 (JP)
(72) Inventor: HASUMI, Shigeru, Otsu-shi Shiga-ken 520 (JP); TANAKA, Kazuo, Gamo-gun Shiga-ken 529-15 (JP); NISHIDOI, Takashi, Yasu-gun Shiga-ken, 520-23 (JP)
(74) Representative: Wilhelms, Rolf E., Dr.
(86) International application number: JP8100195
(87) International publication number: WO8300791

## Description

The present invention relates to a vibratory diaphragm for a loudspeaker. More particularly, it relates to a vibratory diaphragm for use in a loudspeaker of sound appliances such as home stereophonic phonographs, autostereos, television receivers, radios or tape recordè'rs. '

### Background art of the invention

A vibratory diaphragm for a loudspeaker (hereinafter referred to as the "diaphragm"), so far, has mostly been made of paper. The principal reasons why a paper diaphragm has widely been used are; that the raw material is easily obtainable, that relatively flat regenerating frequency characteristics can be obtained because of its high internal loss, and that the efficiency is high because it has a low density and hence is light in weight. However, on the other hand, a paper diaphragm has the disadvantages that sound distortion occurs and the upper regenerating frequency limit is low, because it has a low specific modulus and begins a separation vibration at a relatively low frequency. Moreover, because paper easily absorbs moisture, the paper diaphragm has the disadvantage that the sound quality is influenced by the environment.

On the other hand, a metal diaphragm made of a metal such as beryllium, boron or titanium has a feature that the upper regenerating frequency limit is high, because of the very high specific modulus compared with the paper diaphragm. However, because the metal diaphragm has a very low internal loss, sharp peaks and dips appear in the regenerating frequency characteristics. Moreover, because such metals are inferior in malleability and ductility, they have the disadvantages that it is difficult to form a thin diaphragm and to form a cone- or dome-like shaped diaphragm.

Recently, in contrast with such paper and metal diaphragms, a diaphragm made of filament or fiber reinfroced plastics (hereinafter referred to as the "FRP diaphragm") has been used in some loudspeakers. For example, in the specifications of Japanese patent unexamined publications numbered 59416/78 and 106026/78, an FRP diaphragm made of thermosetting resin such as phenolic or epoxy resin reinforced by carbon filament fabric is described.

This FRP diaphragm has a feature that the specific modulus and the upper regenerating frequency limit are high, because it employs carbon filaments having high specific modulus, especially in the form of a fabric of continuous filaments. However, the internal loss is fairly small compared with the paper diaphragm, though it is larger than that of the metal diaphragm, so that sharp peaks and dips also appear in the regenerating frequency characteristics. Moreover, especially in a loudspeaker having a high input power of more than several tens of watt, heat generation at the voice coil is so great that the temperature at a connection between the voice coil and the diaphragm will be as high as more than 200°C. In such a case, because the aforementioned conventional FRP diaphragm employs a resin of low heat-durability such as phenolic or epoxy resin, the specific modulus of the diaphragm drops and the upper regenerating frequency limit and the sound pressure level especially in the high frequency range of the regenerating frequency characteristic, become lower. The same phenomena is more remarkable when such diaphragms are used for a long time under the burning sun, as in an autostereo or in an autoradio.

On the other hand, in the specification of Japanese patent unexamined publication number 158800/80, a diaphragm made of a composite material composed of polyimide resin and graphite flakes is described. This diaphragm has an internal loss almost equal to that of the paper diaphragm and the specific modulus is also fairly high. Moreover, the drop in the regenerating frequency characteristic caused by heat is of little importance unlike in the aforementioned FRP diaphragm, because the employed polyimide resin has a high heat resistance. However, the diaphragm has a rather fatal disadvantage for a diaphragm in that the mechanical strength is low.

Namely, in order to obtain high specific modulus and large internal loss, this conventional diaphragm contains a lot of graphite flakes, e.g. as much as about 30-90% by volume based on the whole volume. Therefore, the mechanical strength, especially the bending strength and the impact strength, is very low. If the bending strength is low, the diaphragm cracks or in the worst case creaves for large relative displacements generated when each part of the diaphragm moves in different phases in the separation vibration area. Moreover, if the impact strength is low, the diaphragm generates cracks at a sharp rising-up sound, especially with large input power in the lower frequency range.

Further, the diaphragm is generally made in a very thin form so that it is light and has a better efficiency. Usually it is formed in the shape of cone or a dome. Moreover, to improve the regenerating frequency characteristics, ridges or corrugations are often formed. Thus the detailed shape is fairly complicated though its shape is cone- or dome-like as a whole. However, a mixture composed of polyimide resin and a lot of graphite flakes has a poor moldability and tends to break in the manufacturing process. Even when the molding is successful, it is difficult to shape precisely and uniformly in detail. In other words, the diaphragm made of composite material of polyimide resin and graphite flakes lacks equality and uniformity in thickness. Thus, the mechanical strength is much lower.

As mentioned above, conventional diaphragms have advantages and disadvantages in various characteristics such as the specific modulus, the internal loss, the thermal stability, the mechanical strength and the fatigue resistance which are all important for a diaphragm. Therefore, a diaphragm of well-balanced characteristics has been desired.

### Disclosure of the invention

An object of the present invention is to provide a diaphragm of well-balanced characteristics required for a diaphragm, such as the specific modulus, the internal loss, the thermal stability, the mechanical strength and the fatigue resistance.

Another object of the present invention is to provide a diaphragm of low distortion of sound with improved sound quality.

In order to achieve the above objects in accordance with the present invention, a vibratory diaphragm for a loudspeaker made of composite material composed of polyimide resin, graphite granules and fabric of high strength and high modulus filaments, wherein the content of polyimide resin is 35 to 65% by volume, the content of the graphite granules is 5 to 30% by volume and the content of the fabric is 20 to 50% by volume is hereby proposed. The diaphragm of the present invention has superior regenerating frequency characteristics, and has little drop in the characteristics and the sound quality with varying environment or when used for a long time.

### The best mode to carrying out the invention

A diaphragm of the present invention will be explained in detail hereinbelow, with reference to the figures in which

Fig. 1 shows the relationship between the regenerating frequency and the output sound pressure level of loudspeakers, employing a diaphragm of the present invention and a diaphragm made of composite material consisting of polyimide resin and plane weave fabric of glass filaments. Fig. 2 shows the relationship between the regenerating frequency and the second harmonic distortion of loudspeakers using the aforementioned two kinds of diaphragms.

A diaphragm of the present invention is made of composite material composed of polyimide resin, graphite granules and fabric of high strength and high modulus filaments. Namely, this diaphragm is a kind of FRP diaphragm made of a mixture of polyimide resin and graphite granules uniformly dispersed in polyimide resin, which is reinforced by fabric of high strength and high modulus filaments. The mixture will enter into the interior of the textile structure of the fabric and the diaphragm has substantially no pores in it. The diaphragm is in the form of a plate, or is cone- or dome-like. Ridges or corrugations may sometimes be formed. The thickness of the diaphragm is about 0.02-0.7 mm which includes fairly thinner range than that of the most widely used paper ones.

Next, the aforementioned polyimide resin, the graphite granules and the fabric will be explained.

Polyimide resin gives the desired shape to the diaphragm and principally improves the thermal stability and the mechanical strength of the diaphragm. This polyimide resin is most preferably a homopolymer or copolymer of bismaleimide. As such polyimide is obtained through an addition polymerization, no volatile substance generates during the molding process, and pores hardly remain in the diaphragm. Moreover, as the flowability during the molding is high, the dispersability of graphite granules and the impregnatability in to the fabric are superior. Accordingly, a diaphragm made with these materials is very uniform: an unevenness in the specific modulus, the mechanical strength and the internal loss is extremely reduced.

In the above, the bismaleimide is, for example, N,N'-ethylene-bismaleimide, N,N'-hexamethylene-bismaleimide, N,N'-metaphenylene-bismaleimide, N,N'-paraphenylenebismaleimide, N,N'-p,p'-diphenylmethane-bismaleimide, N,N'-p,p'-diphenylether-bismaleimide or N,N'-p,p'-dicyclohexylmethanebismaleimide. The compound which is copolymerized is, for example, a polyamine such as 4,4'-diaminodiphenylmethane, a condensation product of aniline and formaldehyde, 4,4'-diaminodiphenylether, 4,4'-diaminodicyclohexylmethane, 4,4'-diaminodiphenylsulphone, metaphenylenediamine . or paraphenylenediamine, a multi-functional cyanic acid ester such as cyanic acid ester of bisphenol-A or its oligomer, a derivative of isocyanuric acid, a vinyl compound, or an epoxy compound.

The polyimide resin may be polymaleimideamine prepared from maleic acid and a polyamine, a polyamideimide prepared from tricarboxylic acid and a polyamine, a polyamideimide prepared from tricarboxylic acid, unsaturated dicarboxylic acid and a polyamine, a polyimide prepared from tetracarboxylic acid and a polyamine (comprising a polyimide which contains unsaturated bonds such as a vinyl or an ethynyl group, as the end group). In the above, the polyamine is, for example, 4,4'-diaminodiphenylmethane, a condensation product of aniline and formaldehyde, 4,4'-diaminodiphenylether, 4,4'-diaminodiphenylsuflone, 4,4'-diaminodicyclohexylmethane, metaphenylenediamine or paraphenylenediamine. The tricarboxylic acid is, for example, trimellitic acid, 3,3',4-benzophenonetricarboxylic acid, 1,4,5-naphthalenetricarboxylic acid or 1,2,4-butanetricarboxylic acid. Further, the unsaturated dicarboxylic acid is, for example, tetrahydrophthalic acid, 5-norbornene-2,3-dicarboxylic acid or methyl-5-norbornene-2,3-dicarboxylic acid. The tracarboxylic acid is, for example, pyromellitic acid, 3,3',4,4'-benzophenonetetracarboxylic acid, 2,3,6,7-naphthalenetetracarboxylic acid, 3,3',4,4'-diphenyl- . tetracarboxylic acid, 3,3',4,4'-diphenylmethanetetracarboxylic acid or 4,4'-hexafluoroisopropylidenebis- phthalic acid.

The graphite granules mainly act to increase the internal loss and to improve the specific modulus of the diaphragm. Both natural and artificial graphite granules may be employed, while a flake-like shape of 1-200 pm in average diameter is preferable. If the average diameter is less than 111m, a sufficient increase in internal loss and an improvement in the specific modulus is not to be expected. On the other hand, graphite granules having an average diameter of more than 200 um cannot disperse well in polyimide resin. When the mixture of the polyimide resin and the graphite granules is impregnated into the fabric, the fabric acts as a kind of filter against the graphite granules. Therefore, if the diameter of the graphite granules is too large, only polyimide resin passes into the interior of the fabric and the graphite granules tend to remain on the surface of the fabric. Then, the internal loss corresponding to the content of the graphite granules cannot be obtained. Moreover, if the graphite granules remain too much on the surface of the fabric, that part becomes brittle and a multiplied fabric tends to delaminate. The most preferable range of average diameter is 5-50 pm.

The fabric mainly improves the specific modulus, the mechanical strength and the fatigue resistance of the diaphragm. The fabric is made of high strength and high modulus filaments such as carbon, glass or polyaramid filaments. In the present invention "filaments" means a bundle of single filaments having a diameter of 3-15 ¡..lm, that is multi-filaments. The fabric is usually made of one kind of filaments. However, it may be made of a combination of two or more kinds of filaments: carbon and glass filaments, carbon and polyaramid filaments, glass and polyaramide filaments, or carbon, glass and polyaramide filaments.

Woven fabric is most preferable because the filaments are straight and improvement in the specific modulus, the mechanical strength and the fatigue resistance becomes higher. In that case, if the filaments largely crimp at the cross point of warps and wefts, the fabric increases in thickness and weight, and the specific modulus and the mechanical strength of the diaphragm become lower, because the cone- or dome-like shaped fabric bends like a corrugated plate. In order to prevent this, the filaments are preferably fine; the cross sectional area is as small as 0.0003-0.1 mm².

The plain weave structure is most preferable for the fabric because it can be made thin and thus a light diaphragm is obtainable, and because, when formed to cone- or dome-like, dislocations take place regularly, if any, so that the specific modulus and the mechanical strength of the diaphragm are uniform. However, other structures such as twill or satin may also be employed. If the weave density is too low, the filaments separate from the mixture of the polyimide resin and the graphite granules. On the other hand, if it is too high, the mixture can hardly enter into the interior of the fabric. In both cases, the mechanical strength of the diaphragm tends to be low. Therefore, it is preferred that the weave density is about 3-40 filaments/cm. More preferably, it is 4-30 filaments/cm.

In the present invention, non-woven fabric may also be employed as fabric. Though the non-woven fabric is often composed of short fibers, an effect of improvement in the specific modulus and the mechanical strength of the diaphragm is not as high as with the woven fabric, because the short fibers are discontinuous. Therefore, as will be mentioned later, in many cases, it is not employed alone but is employed together with the woven fabric. In case of the non-woven fabric using long filaments, this is not the case.

The fabric may be employed in a single ply or in multiple sheets. In the latter case, the fabric which is laminated may be of the same kind or different kind(s) of filaments. For example, in a three-layered structure consisting of carbon filaments (which has a relatively high specific modulus) covered on both sides of the center fabric of glass or polyaramid filaments (which has a relatively high internal loss), the potential merits of the individual fabric simultaneously appear. Moreover, the lamination of the different weave structures is also preferable. For example, in a three-layered structure consisting of woven fabric on both sides of the center non-woven fabric, the short fibers of the non-woven fabric move into the openings of the woven fabric so as to adhere them firmly together. The layers hardly separate from each other and the mechanical strength as well as the fatigue resistance of the diaphragm are improved.

Next, the content of polyimide resin, the graphite granules and the fabric compared with the whole diaphragm will be explained.

Polyimide resin is the matrix material of the diaphragm as mentioned above and improves mainly the thermal stability and the mechanical strengths. For this purpose, its content is preferably more than 35% by volume. However, if it is too much, an effect of improvement in the specific modulus, the mechanical strength and the fatigue resistance drops and an effect of increase in the internal loss is also reduced, for the relative content ofthefabric and the graphite granules becomes lower. Therefore, it is preferred that the content is under 65% by volume.

If the graphite granules are over 5% by volume, the internal loss is improved fairly well: it increases proportionally up to about 30% by volume. However, if it becomes over 30% by volume, the increase is saturated, while it causes a poor dispersability. Accordingly, it is preferred that the content of graphite granules is 5-30% by volume.

Further, it is preferred that the content of the fabric is 20-50% by volume, though depending on the kind of the filaments, the form or the structure. Namely, if it is less than 20% by volume, an effect of improvement in the specific modulus, the mechanical strength and the fatigue resistance of the diaphragm is small. And if it is over 50% by volume, the thermal stability and the internal loss remain unimproved, for the relative content of the polyimide resin and the graphite granules become lower.

Manufacture of the diaphragm of the present invention may be conducted as follows. After the mixture of the polyimide resin and the graphite granules, mixed in a desired composition ratio, is impregnated into the fabric, the resulted prepreg is put into a mold of the desired form such as a cone-like shape and is pressed at an elevated temperature. If a belt-like fabric is impregnated with the mixture and is then supplied to the molding machine, diaphragms will conveniently and commercially be manufactured.

As detailed above, the diaphragms of the present invention is made of composite material consisting of polyimide resin, graphite granules and fabric of high strength and high modulus filaments. The polyimide resin mainly improves the thermal stability and the mechanical strengths of the diaphragm, the graphite granules mainly increase the internal loss and improve the specific modulus, and the fabric improves the specific modulus, the mechanical strengths and the fatigue resistance. It is to be noted that they cooperate with each other. Accordingly, the diaphragm of the present invention can meet all requirements such as the specific modulus, the internal loss, the mechanical strength, the thermal stability and the fatigue resistance in a well-balanced manner, and any particular characteristic is neither too high nor too low. Thus, with the diaphragm of the present invention, not only the low distortion and high sound quality but also a hard subject of keeping a good sound quality during a very long time in varying environments are now achieved.

### Example 1

Seventy-eight and a half weight parts of 4,4'-diaminodiphenylmethane bismaleimide and 21.5 weight parts of 4,4'-diaminodiphenylmethane were dissolved in 67.0 weight parts ofN-methylpyrrolidone. The solution was then heated at 130°C for 20 minutes. A 40% by weight solution of polyimide (copolymer of bismaleimide) having a viscosity of 20 poises at 23°C was obtained.

Then, 70 weight parts of flake-like natural graphite granules CP, manufactured by Nippon Kokuen Co., Ltd., were added into 100 weight parts of the polyimide solution and stirred with a mixer for 1 hour. An average diameter of the graphite granules was about 7 um.

The solution of polyimide containing the graphite granules was then impregnated to a plain weave fabric WE-116E of glass filaments, manufactured by Nitto Boseki Co., Ltd., by using a wire-bar coater. It was further heated for 20 minutes in a hot-air dryer maintained at 130°C, giving a prepreg of woven fabric. The thickness of the plain weave fabric of glass filaments was about 0.1 mm, and warp and weft densities were about 23 filaments/cm and 25.5 filaments/cm, respectively.

Two square sheets of 25x25 cm were cut out of the prepreg of the woven fabric, which were placed rectangularly so that the warp filaments of each sheet crossed at a right angle. The laminated sheets were put into a cone-like mold and maintained for 30 minutes under a pressure of 50 kg/cm² at 200°C. Thus, a conical diaphragm of the present invention having about 121 mm in outer diameter, about 20 mm in inner diameter, about 26 mm in depth and about 0.22 mm in thickness was obtained. The diaphragm was composed of about 49% of polyimide resin, about 20% of graphite granules and about 31 % of plain weave fabric of glass filaments, all by volume.

A loudspeaker was then obtained by adhering a polyurethane sponge edge and a voice coil and by further equipping a frame to the diaphragm. Hereinafter, the loudspeaker is called as the Example.

The Example was then installed in a closed enclosure having an inner volume of 45 liters, where the regenerating frequency characteristics was measured according to Japanese Industrial Standard JIS C 5531. The result is shown by a full line in Fig. 1. In Fig. 1, F in abscissa is an output sound pressure level and P in ordinate is a frequency.

For comparison, by using the solution of polyimide without graphite granules, a composite diaphragm made of about 61.2% of polyimide resin and about 38.8% of plain weave fabric of glass filaments by volume was prepared similarly. Further, a loudspeaker using the diaphragm was prepared likewise. Hereinafter, the loudspeaker is called as the Comparative. The loudspeaker was then installed in an enclosure where the regenerating frequency characteristics was measured by the same condition as in the Example. The result is shown by a dotted line in Fig. 1.

It is clear from Fig. 1 that the regenerating frequency characteristics of the loudspeaker using the diaphragm of the present invention, namely the Example, are very smooth with few sharp peaks and dips, compared with the loudspeaker using the diaphragm composed only of polyimide resin and the plain weave fabric of glass filaments, namely the Comparative. This shows that a considerable increase in the internal loss of the diaphragm is realized by the use of only such a small amount of graphite granules as 20% by volume. Moreover, the upper regenerating frequency limit of the Comparative is much lower than the Example. The upper regenerating frequency limit is a function of the specific modulus of the diaphragm, while the modulus mainly depends on fabric of glass filaments. Accordingly, it is presumed that there is some unexpected effect of graphite granules when they are used in addition to the plain weave fabric of glass filaments, for both the Example and the Comparative use fabric.

To confirm the above, test pieces of 2 cm wide and 10 cm long were cut from the material used in the Example and the Comparative. Then, the internal loss and the sound speed which is an index of the specific modulus were measured with respect to the test pieces. The measurement was conducted by giving a free damping vibration to each test piece fixed at one end and observing it with an oscilloscope.

As the result of the measurement at room temperature, the internal loss of the Example was about 0.030 and the sound speed was about 3800 m/sec. At 200°C, these values were about 0.049 and about 3550 m/sec, respectively. Namely, it is to be understood that both the internal loss and the sound speed are fairly high, even at a higher temperature. In contrast to this, the sound speed of the Comparative was about 3400 m/sec, a similar value compared with that of the Example, but the internal loss was as small as about 0.006.

The bending strength of the same test pieces was then measured with Tention-bending Tester "Autograph" IS-5000, manufactured by Shimadzu Corporation, to give about 50 kg/mm² for the test piece of the Example, while for the test piece of the Comparative it was about 55 kg/mm², a little less than that of the test piece of the Example. However, this will be enough for practical use.

To determine how the above characteristics of the diaphragm of the Example and the Comparative affect distortion characteristics, the second harmonic distortion was then measured by the method of Japanese Industrial Standard JIS C 5531, the result being shown in Fig. 2. In Fig. 2, F in abscissa and S in ordinate are the frequency and the second harmonic distortion, respectively. From Fig. 2, the second harmonic distortion of the Example shown by a full line is improved compared with that of the Comparative shown by a dotted line.

### Example 2

By the same method as in Example 1 but employing plain weave fabric #6142 of carbon filaments, manufactured byToray Industries, Inc., a conical diaphragm composed of about 42.0% of polyimide resin, about 20.2% of graphite granules and about 37.8% of plain weave fabric of carbon filaments by volume was prepared. The thickness of this diaphragm was about 0.31 mm. The thickness of the plain weave fabric of carbon filaments was about 0.15 mm and the weave densities were about 8.9 filaments/cm in both warp and weft directions.

The internal loss, the sound speed and the bending strength measured by the same methods as in Example 1 with respect to this diaphragm were about 0.032, about 4100 m/sec and about 100 kg/mm², respectively.

## Claims

1. A vibratory diaphragm for a loudspeaker made of composite material composed of polyimide resin, graphite granules and fabric of high strength and high modulus filaments, wherein the content of polyimide resin is 35-65% by volume, the content of the graphite granules is 5-30% by volume and the content of the fabric is 20-50% by volume.

2. A vibratory diaphragm for a loudspeaker as claimed in claim 1, wherein the thickness is 0.02-0.7 mm.

3. A vibratory diaphragm for a loudspeaker as claimed in claim 1, wherein the polyimide resin is a polymer of bismaleimide.

4. A vibratory diaphragm for a loudspeaker as claimed in claim 3, wherein the bismaleimide is N,N'-ethylene-bismaleimide, N,N'-hexamethylene-bismaleimide, N,N'-mataphenylene-bismaleimide, N,N'-paraphenylene-bismaleimide, N,N'-p,p'-diphenylmethane-bismaleimide, N,N'-p,p'-diphenylether- bismaleimide or N,N'-p,p'-dicyclohexylmethane-bismaleimide.

5. A vibratory diaphragm for a loudspeaker as claimed in claim 1, wherein the polyimide resin is a copolymer of bismaleimide.

6. A vibratory diaphragm for a loudspeaker as claimed in claim 5, wherein the copolymerized compound is 4,4'-diaminodiphenylmethane, condensation product of aniline and formaldehyde, 4,4'-diaminodiphenylether, 4,4'-diaminodicydohexylmethane, 4,4'-diaminodiphenylsulfone, metaphenylenediamine, paraphenylenediamine, cyanic acid ester of bisphenol-A or their oligomer, derivative of isocyanuric acid, vinyl compound or epoxy compound.

7. A vibratory diaphragm for a loudspeaker as claimed in claim 5, wherein the bismaleimide is N,N'-ethylene-bismaleimide, N,N'-hexamethylene-bismaleimide, N,N'-metaphenylene-bismaleimide, N,N'-paraphenylene-bismaleimide, N,N'-p,p'-diphenylmethane-bismaleimide, N,N'-p,p'-diphenylether- bismaleimide or N,N'-p,p'-dicyclohexylmethane-bismaleimide, and the copolymerized compound is 4,4'-diaminodiphenylmethane, condensation product of aniline and formaldehyde, 4,4'-diaminodiphenylether, 4,4'-diaminodicyclohexylmethane, 4,4'-diaminodiphenylsulfone, metaphenylenediamine, paraphenylenediamine, cyanic acid ester of bisphenol-A or their oligomer, derivative of isocyanuric acid, vinyl compound or epoxy compound.

8. A vibratory diaphragm for a loudspeaker as claimed in claim 1, wherein the average diameter of the graphite granules is 1-200 pm.

9. A vibratory diaphragm for a loudspeaker as claimed in claim 8, wherein the average diameter of the graphite granules is 5-50 pm.

10. A vibratory diaphragm for a loudspeaker as claimed in claim 1, wherein the fabric is woven fabric.

11. A vibratory diaphragm for a loudspeaker as claimed in claim 10, wherein the woven fabric is plain weave fabric, twill weave fabric or satin weave fabric.

12. A vibratory diaphragm for a loudspeaker as claimed in claim 10, wherein the woven fabric is made of at least one kind of filaments selected from the group consisting of carbon, glass and polyaramid.

13. A vibratory diaphragm for a loudspeaker as claimed in claim 10, wherein the weave density of the woven fabric is 3-40 filaments/cm.

14. A vibratory diaphragm for a loudspeaker as claimed in claim 13, wherein the weave density of the woven fabric is 4-30 filaments/cm.

15. A vibratory diaphragm for a loudspeaker as claimed in claim 1, wherein the cross sectional area of the filament is 0.0003-0.1 mm².

16. A vibratory diaphragm for a loudspeaker as claimed in claim 1, wherein the fabric is non-woven fabric.

## Patentansprüche

1. Vibrierende Platte für Lautsprecher aus Compositwerkstoff, zusammengesetzt aus Polyimidharz, Graphitgranulat und Textilmaterial aus Fasern großer Festigkeit und hohen Moduls, wobei der Gehalt an Polyimidharz 35 bis 65 Volumenprozent, der Gehalt an Graphitgranulat von 5 bis 30 Volumenprozent und der Gehalt an Textilmaterial 20 bis 50 Volumenprozent betragen.

2. Vibrierende Platte für Lautsprecher gemäß Anspruch 1, wobei die Dicke 0.02-0.7 mm beträgt.

3. Vibrierende Platte für Lautsprecher nach Anspruch 1, wobei das Polyimidharz ein Polymer von Bismaleimid ist.

4. Vibrierende Platte für Lautsprecher nach Anspruch 3, wobei das Bismaleimid N,N'-Äthylen-bismaleimid, N,N'-Hexamethylen-bismaleimid, N,N'-Methaphenylen-bismaleimid, N,N'-Paraphenylen- bismaleimid, N,N'-p,p'-Diphenylmethan-bismaleimid, N,N'-p,p'-Diphenyläther-bismaleimid oder N,N'- p,p'-Dicyklohexyimethane-bismaleimid ist.

5. Vibrierende Platte für Lautsprecher nach Anspruch 1, wobei das Polyimidharz ein Copolymer von Bismaleimid ist.

6. Vibrierende Platte für Lautsprecher nach Anspruch 5, wobei die copolymerisierte Verbindung 4,4'-Diaminodiphenylmethan, das Kondensationsprodukt von Anilin und Formaldehyd, 4,4'-Diaminodiphenyläther, 4,4'-Diaminodicyklohexylmethan, 4,4'-Diaminodiphenylsulfon, Methaphenylendiamin, Paraphenylendiamin, Zyansäureester des Bisphenol-A oder deren Oligomere, Derivat der Isozyanursäure, eine Vinylverbindung oder eine Epoxiverbindung ist.

7. Vibrierende Platte für Lautsprecher nach Anspruch 5, wobei das Bismaleimid N,N'- Äthylenbismaleimid, N,N'-Hexamethylen-bismaleimid, N,N'-Methaphenylenbismaleimid, N,N'-Para- phenylen-bismaleimid, N,N'-p,p'-Diphenylmethan-bismaleimid, N,N'-p,p'-Diphenyiäther-bismaleimid oder N,N'-p,p'-Dicyklohexylmethan-bismaleimid und die copolymerisierte Verbindung 4,4'-Diaminodiphenylmethane, Kondensationsprodukt von Anilin und Formaldehyd, 4,4'-Diaminodiphenyläther, 4,4'-Diaminodicyklohexylmethane, 4,4'-Diaminodiphenylsulfon, Methaphenylendiamin, Paraphenylendiamin, Zyansäureester des Bisphenol-A oder deren Oligomere, Derivat von Isozyanursäure, eine Vinylverbindung oder eine Epoxiverbindung sind.

8. Vibrierende Platte für Lautsprecher gemäß Anspruch 1, wobei der durchschnittliche Durchmesser des Graphitgranulats 1-200 pm beträgt.

9. Vibrierende Platte für Lautsprecher gemäß Anspruch 8, wobei der durchschnittliche Durchmesser des Graphitgranulats 5-50 pm beträgt.

10. Vibrierende Platte für Lautsprecher gemäß Anspruch 1, wobei das Textilmaterial ein Textilgewebe ist.

11. Vibrierende Platte für Lautsprecher gemäß Anspruch 10, wobei das Textilgewebe Flachgewebe, Twillgewebe oder Satingewebe ist.

12. Vibrierende Platte für Lautsprecher gemäß Anspruch 10, wobei das Textilgewebe aus mindestens einer der Faserarten Kohlenstoffasern, Glassfasern und Polyaramidfasern hergestellt ist.

13. Vibrierende Platte für Lautsprecher gemäß Anspruch 10, wobei die Webdichte 3-40 Fäden (Faser)/cm beträgt.

14. Vibrierende Platte für Lautsprecher gemäß Anspruch 13, wobei die Webdichte des Textilgewebes 430 Fäden (Fasern)/cm beträgt.

15. Vibrierende Platte für Lautsprecher gemäß Anspruch 1, wobei die Querschnittsfläche der Fasern 0,0003-0,1 mm² beträgt.

16. Vibrierende Platte für Lautsprecher gemäß Anspruch 1, wobei das Textilmaterial nicht gewebt ist.

## Revendications

1. Membrane vibrante pour haut-parleur réalisée en matériau composite constitué d'une résine de polyimide, de granules de graphite et d'un tissu en filaments ayant une grande résistance et un module élevé, où la teneur en résine de polyimide est 35-65% en volume, la teneur en granules de graphite est 5-30% en volume et la teneur en tissu est 20-50% en volume.

2. Membrane vibrante pour haut-parleur selon la revendication 1, où l'épaisseur est 0,02-0,7 mm.

3. Membrane vibrante pour haut-parleur selon la revendication 1, où la résine de polyimide est un polymère de bismaleimide.

4. Membrane vibrante pour haut-parleur selon la revendication 3, où la bismaleimide est la N,N'-éthylène-bismaleimide, la N,N'-héxaméthylène-bismaleimide, la N,N'-metaphénylène-bismaleimide, la N,N'-paraphénylène-bismaleimide, la N,N'-p,p'-diphénylméthane-bismaleimide, la N,N'-p,p'-diphénÿl⁼ ether-bismaleimide ou la N,N'-p,p'-dicyclohexylméthane-bismaleîmide.

5. Membrane vibrante pour haut-parleur selon la revendication 1, où la résine de polyimide est un copolymère de bismaleimide.

6. Membrane vibrante pour haut-parleur selon la revendication 5, où le composé copolymérisé est le 4,4'-diaminodiphénylméthane, un produit de condensation de l'aniline et du formaldéhyde, le 4,4'-diaminodiphénylether, le 4,4'-diaminodicyclohexylméthane, le 4,4'-diaminodiphénylsulfone, la métaphénylènediamine, la paraphénylènediamine, un ester de l'acide cyanique du bisphenol-A ou leur oligomère, un dérivé de l'acide isocyanurique, un composé de vinyle ou un composé époxy.

7. Membrane vibrante pour haut-parleur selon la revendication 6, où la bismaleimide est la N,N'-éthylène-bismaleimide, la N,N'-hexaméthylène-bismaleimide, la N,N'-métaphénylène-bismaleimide, la N,N'-paraphénylène-bismaleimide, la N,N'-p,p'-diphénylméthane-bismaleimide, la N,N'-p,p'-diphényl- ether-bismaleimide ou la N,N'-p,p'-dicyclohéxylméthane-bismaleimide, et le composé copolymérisé est le 4,4'-diaminodiphénylméthane, un produit de condensation de l'aniline et du formaldéhyde, le 4,4'-diaminodiphénylether, le 4,4'-diaminodicyciohexy!méthane, le 4,4'-diaminodiphénylsulfone, la métaphénylènediamine, la paraphénylènediamine, un ester de l'acide cyanique du bisphénol-A ou leur oligomère, un dérivé de l'acide isocyanurique, un composé de vinyle ou un composé epoxy.

8. Membrane vibrante pour haut-parleur selon la revendication 1, où le diamètre moyen des granules de graphite est 1-200 microns.

9. Membrane vibrante pour haut-parleur selon la revendication 8, où le diamètre moyen des granules de graphite est de 5-50 microns.

10. Membrane vibrante pour haut-parleur selon la revendication 1, où le tissu est un tissu tissé.

11. Membrane vibrante pour haut-parleur selon la revendication 10, où le tissu tissé est un tissu à armure toile, un tissu à armure croisée ou un tissu à armure satin.

12. Membrane vibrante pour haut-parleur selon la revendication 10, où le tissu tissée est constitué d'au moins un type de filaments choisi dans le groupe constitué du carbone, du verre et d'un polyaramide.

13. Membrane vibrante pour haut-parleur selon la revendication 10, où la densité de tissage du tissu tissé est 3-40 filaments/cm.

14. Membrane vibrante pour haut-parleur selon la revendication 13, où la densité de tissage du tissu tissé est 4-30 filaments/cm.

15. Membrane vibrante pour haut-parleur selon la revendication 1, où la surface en coupe du filament est 0,0003-0,1 mₘ².

16. Membrane vibrante pour haut-parleur selon la revendication 1, où le tissu est un tissu non tissé.
